

## 1

3,608,297

## SYNTHETIC FILAMENT YARN

Malcolm Carnie Cobb, Anthony Charles Davis, and Kazimierz Wiktor Mieszkis, Pontypool, England, assignors to Imperial Chemical Industries Limited, London, England

No Drawing. Filed May 19, 1969, Ser. No. 826,017  
Claims priority, application Great Britain, May 24, 1968,

24,933/68

Int. Cl. D02g 3/04, 3/22

U.S. CL. 57—140

8 Claims

## ABSTRACT OF THE DISCLOSURE

A yarn comprising a blend of not less than 70% of delustered filaments and not more than 30% of bright filaments wherein the delustered filaments contain not less than 0.7% by weight of a delustrant ( $TiO_2$ ) and the bright filaments contain less than 0.3% of said delustrant.

The present invention relates to improvements in synthetic filament yarns and is especially concerned with the improvement in appearance of yarns heavily delustered to give anti-soiling effects.

The anti-soiling effect of highly delustered yarns using, for example, titanium dioxide, is well known; however, when such yarns are dyed they acquire a rather unpleasant, chalky frequently called dead, appearance. This chalky appearance frequently militates against their use in certain end products, especially carpets where not only is an anti-soiling effect desirable but also bright shiny colours are required.

Since the chalky appearance of the yarn becomes evident at loadings of delustrant below that required to give significant anti-soiling effects, a compromise between the anti-soiling effect, at high delustrant level, and chalkiness of colour is almost impossible to achieve. Thus, for example, when using titanium dioxide as the delustrant in polyamides, chalkiness makes its appearance at a level of about 0.5% whereas a significant anti-soiling effect is evident only above 0.7%.

We have now found, however, that a small percentage of very bright filaments blended with a heavily delustered yarn can break down this chalky background and give a brighter surface appearance, especially when utilised in carpets.

Accordingly therefore, the present invention provides a yarn comprising not less than 70% of delustered fila-

## 2

ments containing not less than 0.7% by weight of a delustrant and not more than 30% of bright filaments containing less than 0.3% of the delustrant.

The term filament includes both continuous filaments and filaments in staple fibre form.

Preferably the delustrant is titanium dioxide and the smaller proportion of yarn contains not more than 0.05% by weight of this delustrant.

The present invention is especially applicable to polyamide yarns and the polyhexamethylene adipamide yarns in particular.

A polyamide yarn suitable for use in carpets comprises 85% of filaments containing 1% titanium dioxide and 15% of filaments containing 0.02% of titanium dioxide.

Blending is most satisfactorily achieved when the filaments are in staple fibre form. Blending may, however, be carried out using continuous filament yarns by doubling especially at spinning, for example. The unevenness of blending which may result from doubling is improved by subjecting the yarns to a bulking treatment e.g. stuffer box crimping, which treatment is normal procedure for carpet yarns of both staple fibres and continuous filaments.

The bright, sparkling effect of the filaments containing the smaller proportion of titanium dioxide, that is the "bright" filaments, may be enhanced by using filaments having a trilobal cross-section. A preferred yarn comprises a blend of polyhexamethylene adipamide staple fibres in which one component, forming 80% by weight of the yarn, has a circular cross-section and contains 1%  $TiO_2$ , and the other component, forming the remaining 20% of the yarn, has a trilobal cross-section and contains 0.02%  $TiO_2$ .

Yarns may advantageously comprise filaments having different deniers within either or both components.

The invention also includes carpets formed from the above-mentioned yarns.

The invention is illustrated by the following examples.

## EXAMPLE 1

6 samples of carpets, A, B, C, D, E and F, were prepared. 3 samples, A, B, C, were made from polyhexamethylene adipamide staple fibre yarns in a cut pile tufted construction, and the other 3, D, E and F, from continuous filament polyhexamethylene adipamide yarns, bulked by the well known stuffer-box crimping technique. Details of the carpets and of yarn construction are given in Table 1.

TABLE 1

| Carpet identification | Yarn count                                                                                                                           | Type of yarn used                                                                             | Percent of the delustered component                                                                         | Percent of the bright component |
|-----------------------|--------------------------------------------------------------------------------------------------------------------------------------|-----------------------------------------------------------------------------------------------|-------------------------------------------------------------------------------------------------------------|---------------------------------|
| A-----                | 2/54 yarn spun on Mackie system from 12 denier 4-6" variable length nylon staple fibre.                                              | 100% nylon staple made from polymer with 1% $TiO_2$ circular cross section.                   | None.                                                                                                       |                                 |
| B-----                |                                                                                                                                      | 100% nylon staple made from polymer with 0.3% $TiO_2$ circular cross section.                 | Do.                                                                                                         |                                 |
| C-----                |                                                                                                                                      | 85% nylon staple made from polymer with 1% $TiO_2$ circular cross section.                    | 15% nylon staple made from polymer with less than 0.02% $TiO_2$ trilobal cross section.                     |                                 |
| D-----                | Continuous filament crimped yarn total denier 3,650,204 filaments.                                                                   | 100% nylon made from polymer with 1% $TiO_2$ circular cross section.                          | None.                                                                                                       |                                 |
| E-----                |                                                                                                                                      | 100% nylon yarn made from polymer with 0.2% $TiO_2$ circular cross section.                   | Do.                                                                                                         |                                 |
| F-----                | Continuous filament crimped yarn folded at crimping from 5 ends of 730/40 making total after crimping of 3,650 denier 200 filaments. | 80% of nylon yarn from polymer with 1% $TiO_2$ in four ends of 730/40 circular cross section. | 20% of nylon yarn made from polymer with 0.02% $TiO_2$ in form of one end of 730/40 trilobal cross section. |                                 |

These carpets were dyed in 3 colours, namely, golden yellow, red and dark green. Comparisons of the colours of the carpets showed that A and D were always less bright than the remaining B, C and E, F. The differences in brightness between carpets B and C or E and F were very small in all cases. Thus the addition of a small amount of a brighter component in a yarn with a high titanium dioxide content provides a degree of brightness similar to that obtained with yarns of generally low total delustrant content B and E.

Samples of the above carpets in the white, undyed state were laid in a corridor carrying a large volume of traffic. After a period of 2 months, differences in rate of soiling were apparent. The carpets formed from the yarns containing a low total delustrant content, B and E, showed a significantly greater degree of soiling than the four carpets A and C or D and F, which were formed from yarns containing high delustrant content. The differences in soiling between carpets A and C or between D and F were marginal.

#### EXAMPLE 2

4 carpets, G, H, I and K, were made from polyhexamethylene adipamide staple fibre yarn in a cut pile tufted construction; details of the carpets and yarn construction are given in Table 2.

These carpets were dyed in each of 3 colours, namely, golden yellow, red and dark green. Comparison of colours of these carpets showed that carpets L and M were much less bright than N and O. The difference in brightness between carpets N and O was small but carpet O was slightly brighter. In this case the increase in brightness obtained by addition of 33% of yarn with the delustrant content of 0.2% was smaller than that obtained with 15% and 20% of yarn with almost nil delustrant content (i.e. less than 0.02%  $TiO_2$ ) quoted in Examples 1 and 2 above respectively.

Samples of the above carpets in the white undyed state were laid in a corridor carrying a large volume of traffic for 90 working days.

The difference in soiling by visual observation was apparent after 30 days. Carpets L and M appeared cleaner than N and O. The difference between L and M was very small, carpet N was slightly more dirty, and carpet O was definitely worst. After 90 days of wear, carpet L and M were still significantly cleaner than N and O but the difference between N and O had almost disappeared.

The soiling of these carpets was measured using SAD (soiling additional density) method described by J. Lord and W. H. Reese in the Journal of Textile Institute 1960, vol. 51, T.419, where  $SAD = \log R_o/R_s$ ,  $R_o$  being percent

TABLE 2

| Carpet identification | Type of yarn used                                                               |                                                                               |                                                                                    |
|-----------------------|---------------------------------------------------------------------------------|-------------------------------------------------------------------------------|------------------------------------------------------------------------------------|
|                       | Percent and type of delustrant component                                        | Percent and type of bright component                                          | Yarn count and construction                                                        |
| G-----                | 80% nylon staple made from polymer with 1% $TiO_2$ , trilobal cross section.    | 20% nylon staple made from polymer with 0.01% $TiO_2$ trilobal cross section. | 2/44 yarn spun on Mackie system from 12 denier variable length 4"-6" staple fibre. |
| H-----                | 80% nylon staple made from polymer with 1.3% $TiO_2$ , trilobal cross section.  | 20% nylon staple made from polymer with 0.01% $TiO_2$ trilobal cross section. | Do.                                                                                |
| I-----                | 100% nylon staple made from polymer with 1% $TiO_2$ , trilobal cross section.   | None.                                                                         | Do.                                                                                |
| K-----                | 100% nylon staple made from polymer with 0.3% $TiO_2$ , circular cross section. | do                                                                            | Do.                                                                                |

These carpets were dyed in each of 3 colours, namely, golden yellow, red and dark green. Comparison of colours of these carpets showed that carpet I was less bright than the remaining G, H and K. The differences in brightness between carpets G H and K were small in all cases. Thus the addition of a small amount of a brighter component in a yarn with a high  $TiO_2$  content G and H provides a degree of brightness similar to that obtained with yarns of generally low total delustrant content K.

Samples of the above carpets in the white undyed state were laid in a corridor carrying a large volume of traffic. After a period of 2 months, differences in rate of soiling were apparent. The carpet made from yarn with low total delustrant content K showed a significantly greater degree of soiling than the three carpets G, H and I made from yarns with higher average delustrant contents. The differences in soiling between carpets G, H and I were marginal.

#### EXAMPLE 3

4 carpets, L, M, N and O were made from polyhexamethylene adipamide continuous filament undyed in a cut pile tufted construction. Details of the carpets and yarn construction are given in Table 3.

green reflectance of light measured in a clean carpet circle and  $R_s$  being the same measurement on a circle from soiled carpet. The instrument used was the Colormaster Model V made by Meeco Instrument Manufacturers, Engineering & Equipment Corporation, Warrington, Pa., U.S.A. For each case two circles were tested and an average value for SAD taken. Table 4 shows the results for L, M, N and O carpets measured after 24 and 90 soiling days.

TABLE 4

| Number of soiling days | SAD for carpets |       |       |       |
|------------------------|-----------------|-------|-------|-------|
|                        | L               | M     | N     | O     |
| After 24 days-----     | 0.282           | 0.255 | 0.271 | 0.296 |
| After 90 days-----     | 0.314           | 0.300 | 0.334 | 0.333 |

The instrument assessment of soiling confirms the visual assessment that L and M carpets were cleaner than N and O and that the advantage of N carpet (blended yarn) over O carpet made of 100% low delustrant yarn after 24 days disappeared after more prolonged soiling. This experiment shows also that for high delustrant content yarns the effect of cross-section, trilobal versus circular, is small.

TABLE 3

| Carpet identification | Type of yarn used                                                                                                                    |                                                                                                                                          |                                                                                                                                                         |
|-----------------------|--------------------------------------------------------------------------------------------------------------------------------------|------------------------------------------------------------------------------------------------------------------------------------------|---------------------------------------------------------------------------------------------------------------------------------------------------------|
|                       | Percent and type of delustrant component                                                                                             | Percent and type of bright component                                                                                                     | Yarn count and construction                                                                                                                             |
| L-----                | 100% nylon yarn made from polymer with 1% $TiO_2$ , trilobal cross section.                                                          | None.                                                                                                                                    | Continuous filament crimped yarn total denier 3,650 with 204 filaments.                                                                                 |
| M-----                | 100% nylon yarn made from polymer with 1% $TiO_2$ , circular cross section.                                                          | do                                                                                                                                       |                                                                                                                                                         |
| N-----                | Approximately 67% of nylon yarn made from polymer, with 1% $TiO_2$ , in 2 ends of 1,210 denier 68 filaments, trilobal cross section. | Approximately 33% of nylon yarn made from polymer with 0.2% $TiO_2$ , in one end of 1,210 denier 68 filaments of trilobal cross section. | Continuous filament crimped yarn folded at crimping from 3 ends of 1,210 denier 68 filaments making total after crimping of 3,630 denier 204 filaments. |
| O-----                | 100% nylon yarn made from polymer with 0.2% $TiO_2$ , trilobal cross section.                                                        | None.                                                                                                                                    | Continuous filament crimped yarn made from 3,650 denier 204 filaments.                                                                                  |

**5**  
EXAMPLE 4

3 carpets P, R and S were made from polyhexamethylene adipamide staple fibre yarn in a cut pile tufted construction; details of the carpets and yarn construction are given in Table 5.

**6**

3. A yarn according to claim 2 wherein the polyamide is polyhexamethylene adipamide.
4. A yarn according to claim 1 wherein the delustrant is titanium dioxide and the bright yarn contains not more than 0.05% by weight of this delustrant.

TABLE 5

| Carpet identification | Type of yarn used                                                                                                       |                                                                                       |                                                                   |
|-----------------------|-------------------------------------------------------------------------------------------------------------------------|---------------------------------------------------------------------------------------|-------------------------------------------------------------------|
|                       | Percent and type of delusted component                                                                                  | Percent and type of bright component                                                  | Yarn count and construction                                       |
| P-----                | 18 denier 10%, 16 denier 70%, 12 denier 20%, all made from polymer with 1% TiO <sub>2</sub> , circular cross section.   | None-----                                                                             | 2/54 yarn spun on Mackie system from variable 4"-6" staple fibre. |
| R-----                | 18 denier 10%, 16 denier 68%, all made from polymer with 1.3% TiO <sub>2</sub> , circular cross section.                | 12 denier 22% made from polymer with 0.01% TiO <sub>2</sub> , trilobal cross section. |                                                                   |
| S-----                | 18 denier 10%, 16 denier 70%, 12 denier 20%, all made from polymer with 0.2% TiO <sub>2</sub> , circular cross section. | None-----                                                                             |                                                                   |

These three carpets were dyed in each of 2 colours, 20 namely, pink and yellow golden.

In comparison, carpet P was much duller and less shiny than carpets R and S. The difference in brightness between carpets R and S was small. Thus the addition of a small amount of a brighter component with practically nil delustrant R to yarn with high delustrant content provides a degree of brightness similar to that obtained with yarn with a low total delustrant content S.

Samples of the above carpets in the white, undyed state were laid in a corridor carrying a large volume of traffic. After a period of two months, differences in the rate of soiling were apparent. The carpet made from yarn with low total delustrant content S showed a significant greater degree of soiling than the other two carpets P and R made from yarns with a total high delustrant content. The differences in soiling between carpets R and P were small, with P being marginally better than R.

What we claim is:

1. A yarn comprising not less than 70% of delusted filaments containing not less than 0.7% by weight of a delustrant and not more than 30% of bright filaments containing less than 0.3% by weight of a delustrant.

2. A yarn according to claim 1 wherein the filaments are polyamide filaments.

5. A yarn according to claim 1 wherein the bright filaments have a trilobal cross-section.

6. A yarn according to claim 4 comprising 85% of filaments containing 1% titanium dioxide and 15% filaments containing less than 0.3% by weight of a delustrant.

25 7. A yarn according to claim 5 comprising 80% polyhexamethylene adipamide staple fibres of circular cross-section containing 1% titanium dioxide and 20% polyhexamethylene adipamide staple fibers of trilobal cross-section containing 0.02% titanium dioxide.

30 8. A yarn according to claim 1 wherein the filaments have different deniers.

**References Cited**

UNITED STATES PATENTS

|    |           |         |               |          |
|----|-----------|---------|---------------|----------|
| 35 | 2,913,801 | 11/1959 | Kessler ----- | 28—74(H) |
|    | 3,480,582 | 11/1969 | Brooks -----  | 57—140BY |

DONALD E. WATKINS, Primary Examiner

U.S. CL. X.R.

57—140J